

Patented Feb. 13, 1923.

1,445,173

# UNITED STATES PATENT OFFICE.

WILLIAM H. ROBINSON, OF LOS ANGELES, CALIFORNIA.

## PAINT.

No Drawing.

Application filed March 1, 1922. Serial No. 540,281.

To all whom it may concern:

Be it known that I, WILLIAM H. ROBINSON, a citizen of the United States, and a resident of Los Angeles, in the county of Los Angeles and State of California, have invented new and useful Improvements in Paint, of which the following is a specification.

This invention relates to and has for a main object the provision of a paint particularly adapted for the purpose of coating a surface of canvas or fabric, such as is used for awnings, curtains and the like, whereby the paint may be applied with a uniform and smooth coating over the surface of the fabric, and will be prevented from saturating or working through to the other side of the fabric.

It will be understood that it is frequently desirable to paint or color canvas such as is used in awnings for the purpose of stripping or ornamenting the same, and heretofore it has been found practically impossible to apply a uniform and smooth coating of paint on the canvas without discoloring the inner side of the fabric, and this discoloration makes the fabric unsightly and is generally undesirable.

It is a further object of my invention to provide in combination with an ordinary commercial oil paint, a mixture of wheat flour paste, which when thoroughly mixed with the paint will form a foundation on the surface of the fabric for the paint, and when spread uniformly and evenly over the surface of the fabric will fill in the interstices and prevent the absorption of the oils from the paint by the fabric, and thereby prevent the discoloration of the opposite surface of the fabric.

Another object is to add to the mixture of paint and flour paste, a suitable quantity of drier, such as japan drier, so that the mixture will be quickly dried after an application to the fabric.

In the preparation of my paint I add a certain amount of water in the preparation of the flour paste, and as it is a well-known fact that water and oils do not mix, it is a further object of my invention to add to the other ingredients mentioned a suitable quantity of liquid soap, such as common laundry soap, for the purpose of effecting a complete union of the other ingredients.

Other objects may appear as the description progresses.

In the preparation of my paint I first mix water and wheat flour substantially in the proportion of a half-gallon of water to one pound of flour, and cook the mixture until a thick paste is formed, whereupon a total volume of about  $\frac{1}{3}$  of a pail of paste is provided; thereafter, for paint of ordinary consistency I add about  $3\frac{1}{2}$  pounds minimum quantity of ordinary commercial oil paint to the flour paste and thoroughly mix the paste and paint together by agitation. Then I add approximately  $\frac{1}{2}$  cup of water to  $\frac{3}{4}$  of a cake of common laundry soap and boil the water thoroughly for dissolving the soap therein and add the liquid thus provided to the mixture of paste and paint, and the soap thus added serves to form a perfect union between the paste and oil. Thereafter, for the purpose of quickly drying the paint, after its application to the fabric, I add to the other ingredients mentioned, about  $\frac{1}{4}$  of a pint of japan drier, and thoroughly mix the same therewith.

While it is not necessary that the ingredients be separately prepared and mixed one after the other, as hereinbefore described, it is a convenient way of providing my improved paint and preferable to the mixture of all of the ingredients together, but it will be understood that I may mix all of the said ingredients together if desirable and convenient.

In the preparation of the paint, care should be taken that not too much of the laundry soap is added to the mixture, for the reason that too much alkali would then be provided for accomplishing the result set forth, and the good results would to a certain extent be more or less nullified. The addition of the flour paste, as stated, serves to prevent the paint from permeating the fabric and also renders the mixture easily capable of being spread uniformly and smoothly over a large surface.

My paint composition consists of the several ingredients before mentioned, in substantially the following proportions: Water  $\frac{1}{2}$  gallon, wheat flour 1 pound, oil paint  $3\frac{1}{2}$  pounds, melted soap 8 ounces and japan drier  $\frac{1}{2}$  of a pint; or the same formula may be interpreted into quantities of like denominations, as follows: Water,  $4\frac{1}{4}$  pounds; flour, 1 pound; oil paint,  $3\frac{1}{2}$  pounds; melted soap,  $\frac{1}{2}$  pound, and drier 4 ounces.

Substantially the same result may be accomplished by adding the ingredients in the

2  
following proportions: Water 44.8% flour 101% oil paint 37.1% melted soap 5.1% drier 2.5%. However, inasmuch as the flour and water are mixed as a preliminary to the mixture of the complete composition, the best results may be obtained by the following formula:

5 Wheat flour paste 55.3% oil paint 37.1% melted laundry soap 5.1% and japan drier 10 2.5%.

10 It will be understood that the ingredients of my composition may vary in quality and character in different localities to a more or less extent, and in such case the ingredients 15 stated in the formulae hereinbefore named may of necessity be modified so that more or less of certain of the ingredients may be added for obtaining the best results, and I therefore do not wish to be understood as 20 limiting myself to the definite proportions of the several ingredients hereinabove set forth, nor do I desire to be limited to the exact method stated for mixing the several ingredients together.

25 In the application of my paint to fabric for the purposes cited, usually one coat of the mixture will suffice for ordinary purposes, and the mixture should be of such consistency as to lend itself readily to application to fabric, and probably slightly 30 thicker in consistency than ordinary commercial paint, but the consistency of the mixture will depend to a greater or less extent on the weave of the particular fabric 35 on which the paint is used.

It will be readily understood that fabric of loose weave would require a thicker mixture than would a fabric of close weave, in order that the paint may not saturate 40 through to the opposite side of and tend to discolor the fabric and render the same irregular.

The mixture in the proportions stated 45 lends itself to quick drying when exposed to the air, and is generally found satisfactory for all commercial purposes.

In cases where quick drying is not necessary and where the material painted is not necessarily folded after the painting operation and can be subjected to a slow drying process, I may omit the drier hereinbefore mentioned. I also conceive it to be 50 novel and useful in paints to mix wheat

flour paste with oil paints for the purpose described, and to this end I desire to claim 55 broadly on the mixture of the wheat flour paste with the oil paint for the purpose of preventing the saturation and absorption of the paint by the material. I also consider it possible and occasionally expedient to 60 omit the soap from my composition.

What I claim is:

1. The within described composition consisting of about  $\frac{1}{2}$  gallon of water; 1 pound of wheat flour;  $3\frac{1}{2}$  pounds of oil paint; 8 65 ounces of melted laundry soap, and  $\frac{1}{2}$  pint of drier, as described.

2. The within described composition consisting of cooked wheat flour paste 27%; commercial oil paint 37.1% melted laundry 70 soap 5.1% and japan drier 2.5%, substantially as described.

3. The within described composition including wheat flour paste and commercial oil paint mixed together substantially in the 75 proportions stated.

4. The within described composition including wheat flour paste, commercial oil paint and soap, as described.

5. The within described composition including cooked wheat flour paste, commercial oil paint, and melted laundry soap, substantially in the proportions stated.

6. The within described composition including a relatively pre-ponderant quantity 85 of commercial oil paint and cooked wheat flour paste, added thereto, as and for the purpose stated.

7. The within described composition including commercial oil paint as a predominant 90 ingredient, wheat flour and water formed into a paste and added to the paint, and common laundry soap melted and added to said other ingredients for effecting the complete mixture thereof.

8. The within described composition including commercial oil paint as a predominant 95 ingredient, wheat flour and water formed into a paste and added to the paint, common laundry soap melted and added to 100 said other ingredients for effecting the complete mixture thereof, and japan drier as and for the purpose stated.

WILLIAM H. ROBINSON.

Witness:  
CHAS. BAGG.